

## UNITED STATES PATENT OFFICE.

FRITZ STRAUB, OF BASEL, SWITZERLAND, ASSIGNOR TO THE FIRM "SOCIETY OF CHEMICAL INDUSTRY IN BASLE," OF BASEL, SWITZERLAND.

## PROCESS FOR THE PRODUCTION OF FAST TINTS ON VEGETABLE FIBER.

No Drawing. Application filed May 23, 1927, Serial No. 193,730, and in Switzerland May 27, 1926.

The present invention relates to a process for producing fast tints on vegetable fibers. It comprises the process for producing these fast tints, and the material that has been 5 dyed according to this new process.

It has been found that the chromium compounds of azo-dyestuffs from diazo-compounds which contain in ortho-position to the diazo-group a group adapted to form lakes, 10 such as the OH-group, or the carboxyl group, and which hitherto have been used chiefly for dyeing animal fibers, are also suitable for producing fast tints on vegetable fibers. This result could not be anticipated and is the 15 more surprising, because when wool dyed with chromium compounds is subjected to alkaline fulling in presence of cotton, the latter does not become dyed.

The fulling of wool consists, as is well-known, in treating this material at about 50° C. for a long time in a fulling machine with a fulling liquid containing soap and soda. During this operation there is always passing some dyestuff from the wool fiber into the 25 fulling liquid. Now, if wool, as is frequently the case, is fulled in presence of cotton, then cotton is dyed by the dyestuff which is contained in the alkaline fulling liquid, if this dyestuff has affinity for cotton. It is therefore to be considered as altogether surprising that when wool dyed with chromium compounds of ortho-hydroxy-azo-dyestuffs or ortho-carboxy-azo-dyestuffs is fulled in presence of cotton the latter is not dyed, although 30 it can be smoothly dyed under the conditions of a dyeing bath.

The dyeings produced on vegetable fibers by means of chromium compounds of ortho-hydroxy-azo-dyestuffs or ortho-carboxy-azo-dyestuffs may be distinguished by their very 40 good fastness to light, and by their remarkable fastness to water and washing surprising for direct cotton dyestuffs which, generally, do not possess these properties.

The affinity of the chromium compounds of certain azo-dyestuffs is particularly good for vegetable fibers, namely when the dyestuff is derived from such components as lend to the azo-dyestuff made from them an affinity 45 for cotton. Such components are, among others, the 2:5:7-, the 2:8:6- and the 1:5:7-amino-naphtholsulfonic acids and the derivatives and substitution products thereof; fur-

ther the products which contain the residue of the dehydrothio-p-toluidine, of the primuline, and the like, are particularly suitable. Such products are, for example, the dyestuffs which are obtained from the condensation 55 products of dehydrothiotauidine or of primuline with acetoacetic ester and ortho-hydroxy-diazo-compounds.

The following example illustrates the invention, the parts being by weight:—

## Example.

A dye bath is prepared with 2 parts of the chromium compound of the azo-dyestuff from diazotized 2-amino-4-chloro-5-nitro-1-phenol and 2:5-aminonaphthol-7-sulfonic acid (acid coupling) corresponding with the formula



50 parts of Glauber's salt or 30 parts of common salt. Then 100 parts of cotton are introduced into this bath at 60-70° C., boils up within 1/4 hour and continues dyeing during a further 1/2 to 3/4 hour. The dyed cotton is then rinsed as usual and dried. It is dyed in 80 blue-green tints fast to light. The dyeing may also be conducted in a weakly alkaline or weakly acid bath, if necessary with addition of chromium salts.

The following table gives a range of tints 90 which can be obtained according to the new process:—

| Diazotizing component                       | Coupling component                    | Tint of the direct cotton dyeing | 95  |
|---------------------------------------------|---------------------------------------|----------------------------------|-----|
| 2-amino-1-phenol-4-sulfo-6-carboxylic acid. | Acetoacetic anilide.....              | Greenish yellow.                 |     |
| 2-amino-1-phenol-4-sulfo-6-carboxylic acid. | Acetoacetic- $\alpha$ -naphthylamide. | Greenish yellow                  |     |
| 2-amino-1-phenol-4-sulfo-6-carboxylic acid. | Acetoacetic-p-dichloro-anilide.       | Greenish yellow.                 | 100 |
| 2-amino-1-phenol-4-sulfo-6-carboxylic acid. | Acetoacetic-o-toluide.                | Greenish yellow.                 |     |
| 2-amino-1-phenol-4-sulfo-6-carboxylic acid. | Acetoacetic-o-aniside.                | Greenish yellow.                 |     |
| 1-aminobenzene-2-carboxylic acid.           | Acetoacetic anilide.....              | Yellow.                          | 105 |

| Diazotizing component                                             | Coupling component                                                                                                             | Tint of the direct cotton dyeing   | Diazotizing component                                             | Coupling component                          | Tint of the direct cotton dyeing | 65  |
|-------------------------------------------------------------------|--------------------------------------------------------------------------------------------------------------------------------|------------------------------------|-------------------------------------------------------------------|---------------------------------------------|----------------------------------|-----|
| 2-amino-1-phenol-4-sulfonic acid.                                 | Acetoacetic ester                                                                                                              | Yellow.                            | 2-amino-1-phenol-4-sulfonic acid.                                 | 2:4-diaminodiphenyl ether.                  | Brown.                           |     |
| 5 2-amino-1-phenol-4-chloro-5-sulfonic acid.                      | Acetoacetic ester                                                                                                              | Yellow.                            | 2-amino-1-phenol-4-sulfonic acid.                                 | m-phenylenediamine                          | Brown.                           |     |
| 4-nitro-2-amino-1-phenol                                          | Acetoacetic ester                                                                                                              | Yellow.                            | Nitrated diazo compound of the 1:2-aminonaphthol-4-sulfonic acid. | Acetoacetic-o-xylidide.                     | Brown.                           | 70  |
| 4-chloro-2-amino-1-phenol-6-sulfonic acid.                        | Acetoacetic anilide                                                                                                            | Yellow.                            | Nitrated diazo compound of the 1:2-aminonaphthol-4-sulfonic acid. | Acetoacetic-o-toluidide                     | Brown.                           |     |
| 4-nitro-2-amino-1-phenol-6-sulfonic acid.                         | Acetoacetic anilide                                                                                                            | Yellow.                            | 2-amino-1-phenol-4-sulfonic acid.                                 | 4-chloro-1:3-phenylendiamine                | Brown.                           |     |
| 10 2-amino-1-phenol-4-sulfo-6-carboxylic acid.                    | Acetoacetic-p-chloroanilide                                                                                                    | Yellow.                            | 2-amino-1-phenol-4-sulfonic acid.                                 | m-toluylenediamine                          | Red-brown.                       | 75  |
| 4-nitro-2-amino-1-phenol-6-carboxylic acid.                       | Acetoacetic anilide                                                                                                            | Yellow.                            | Nitrated diazo compound of the 1:2-aminonaphthol-4-sulfonic acid. | Acetoacetic-o-chloroanilide                 | Red-brown.                       |     |
| 2-amino-1-phenol-4-sulfonic acid.                                 | Acetoacetic-p-chloroanilide                                                                                                    | Yellow.                            | Nitrated diazo compound of the 1:2-aminonaphthol-4-sulfonic acid. | Acetoacetic-m-xylidide                      | Red-brown.                       | 80  |
| 2-amino-1-phenol-4-sulfonic acid.                                 | Acetoacetic-o-toluidide                                                                                                        | A red yellow.                      | 2-amino-1-phenol-4-sulfamide.                                     | 2:4-diaminodiphenyl-ether-4'-sulfonic acid. | Red-brown.                       |     |
| 15 2-amino-1-phenol-4-chloro-5-sulfonic acid.                     | Acetoacetic-o-xylidide                                                                                                         | A red yellow.                      |                                                                   |                                             |                                  |     |
| 2-amino-1-phenol-4-chloro-5-sulfonic acid.                        | Acetoacetic ester                                                                                                              | A red yellow.                      |                                                                   |                                             |                                  |     |
| 2-amino-1-phenol-4-chloro-5-sulfonic acid.                        | Acetoacetic anilide                                                                                                            | A red yellow.                      |                                                                   |                                             |                                  |     |
| 2-amino-4-acetylaminophenol-6-sulfonic acid.                      | Acetoacetic ester                                                                                                              | A red yellow.                      |                                                                   |                                             |                                  |     |
| 20 2-amino-1-phenol-4-chloro-5-sulfonic acid.                     | Acetoacetic-m-toluidide                                                                                                        | A red yellow.                      |                                                                   |                                             |                                  |     |
| 2-amino-1-phenol-4-sulfonic acid.                                 | Acetoacetic-o-anisidine                                                                                                        | A red yellow.                      |                                                                   |                                             |                                  |     |
| 2-amino-4-methyl-1-phenol-5-sulfonic acid.                        | Acetoacetic anilide                                                                                                            | A red yellow.                      |                                                                   |                                             |                                  |     |
| 2-amino-1-phenol-4-chloro-6-sulfonic acid.                        | Acetoacetic ester                                                                                                              | A red yellow.                      |                                                                   |                                             |                                  |     |
| 25 2-amino-1-phenol-4-chloro-5-sulfonic acid.                     | Acetoacetic-o-toluidide                                                                                                        | A red yellow.                      |                                                                   |                                             |                                  |     |
| 2-amino-1-phenol-4-sulfamide.                                     | 1-(3-sulfamido)-phenyl-3-methyl-5-pyrazolone.                                                                                  | Orange.                            |                                                                   |                                             |                                  |     |
| 2-amino-4-chloro-1-phenol.                                        | ω-methansulfonic acid of 1-(m-amino)-phenyl-3-methyl-5-pyrazolone.                                                             | Red.                               |                                                                   |                                             |                                  |     |
| 30 1:2-aminonaphthol-4-sulfonic acid (2 molecules).               | Urea of 1-(m-amino)-phenyl-3-methyl-5-pyrazolone (1 mol.).                                                                     | Pink.                              |                                                                   |                                             |                                  |     |
| 1:2-aminonaphthol-4-sulfonic acid (2 molecules).                  | 1-(m-amino)-phenyl-3-methyl-5-pyrazolone.                                                                                      | Pink.                              |                                                                   |                                             |                                  |     |
| 2-amino-1-phenol-4-sulfonic acid.                                 | 1-hydroxynaphthaline-4-phenylketone.                                                                                           | Red-violet.                        |                                                                   |                                             |                                  |     |
| 35 2-amino-1-phenol-4-chloro-5-sulfonic acid.                     | 1-hydroxynaphthaline-4-phenylketone.                                                                                           | Blue-violet.                       |                                                                   |                                             |                                  |     |
| 1:2-aminonaphthol-4-sulfonic acid.                                | α-naphthol                                                                                                                     | A red blue.                        |                                                                   |                                             |                                  |     |
| 2-amino-1-phenol-4-sulfo-6-carboxylic acid.                       | Primary condensation product from 1 mol. 1:2-aminonaphthol-3:6-disulfonic acid and 1 mol. cyanuric chloride.                   | Blue.                              |                                                                   |                                             |                                  | 100 |
| 40 2-amino-4-chloro-5-nitro-1-phenol.                             | β-naphthylamine                                                                                                                | Green.                             |                                                                   |                                             |                                  |     |
| 2-amino-5-nitro-1-phenol.                                         | 2:5-aminonaphthol-7-sulfonic acid (acid coupled).                                                                              | Green.                             |                                                                   |                                             |                                  |     |
| 4:6-dinitro-1-amino-2-phenol.                                     | 2:8-aminonaphthol-6-sulfonic acid.                                                                                             | Olive.                             |                                                                   |                                             |                                  |     |
| 45 4:6-dinitro-1-amino-2-phenol.                                  | 1:8-aminonaphthol-4-sulfonic acid.                                                                                             | Olive.                             |                                                                   |                                             |                                  |     |
| 4:6-dichloro-2-amino-1-phenol.                                    | 2:2'-dinaphthylamin-5:5'-dioxo-7:7'-disulfonic acid.                                                                           | Blue-gray.                         |                                                                   |                                             |                                  |     |
| 2-amino-1-phenol-4-sulfo-6-carboxylic acid.                       | Secondary condensation product from 1 mol. 1:8-aminonaphthol-3:6-disulfonic acid, 1 mol. cyanuric chloride and 1 mol. aniline. | Greenish tinged gray.              |                                                                   |                                             |                                  | 105 |
| 50                                                                | 1-amino-2-p-tolylsulfonic acid (acid coupling); 4:6-dinitro-2-amino-1-phenol (alkaline coupling).                              | 2:5-aminonaphthol-7-sulfonic acid. | Gray.                                                             |                                             |                                  |     |
| 55 2-amino-1-phenol-4-sulfamide.                                  | 1:5-dioxynaphthalin...                                                                                                         | Gray.                              |                                                                   |                                             |                                  |     |
| Nitrated diazo compound of the 1:2-aminonaphthol-4-sulfonic acid. | 5:8-dichloro-1-naphthol.                                                                                                       | Gray.                              |                                                                   |                                             |                                  |     |
| 4-chloroaniline (acid coupling).                                  | 2:5-aminonaphthol-7-sulfonic acid.                                                                                             | Reddish gray.                      |                                                                   |                                             |                                  | 115 |
| 60 4:6-dinitro-2-amino-1-phenol (alkaline coupling).              | Sulfonic acid of the 2:4-diamino-4'-chlorodiphenyl ether.                                                                      | Brown.                             |                                                                   |                                             |                                  |     |
| 4-chloro-2-amino-1-phenol.                                        |                                                                                                                                |                                    |                                                                   |                                             |                                  | 120 |
|                                                                   |                                                                                                                                |                                    |                                                                   |                                             |                                  | 125 |

What I claim is:-

1. Process for the production of fast tints on the vegetable fiber, consisting in dyeing the vegetable fiber from such dyeing baths which have been prepared with chromium compounds of azo-dyestuffs from such diazo compounds which contain in the ortho-position to the diazo group a group adapted to the formation of lakes.

2. Process for the production of fast tints on the vegetable fiber, consisting in dyeing the vegetable fiber from such dyeing baths which have been prepared with chromium compounds of azo-dyestuffs from ortho-hydroxy-diazo compounds.

3. Process for the production of fast tints on the vegetable fiber, consisting in dyeing the vegetable fiber from such dyeing baths which have been prepared with chromium compounds of azo-dyestuffs from ortho-hydroxy-diazo compounds and such coupling components which impart affinity to cotton to the azo-dyestuff derived therefrom.

4. Process for the production of fast tints on the vegetable fiber, consisting in dyeing the vegetable fiber from such dyeing baths which have been prepared with chromium compounds of azo-dyestuffs from ortho-hydroxy-diazo compounds and 2:5-aminonaphthol-7-sulfonic acid compounds.

5. Process for the production of fast tints on the vegetable fiber, consisting in dyeing the vegetable fiber from such dyeing baths which have been prepared with chromium compounds of azo-dyestuffs from ortho-hydroxy-diazo compounds and N-substitution products of the 2:5-aminonaphthol-7-sulfonic acid.

6. Process for the production of fast tints on the vegetable fiber, consisting in dyeing the vegetable fiber from such dyeing baths which have been prepared with chromium

compounds of azo-dyestuffs from ortho-hydroxy-diazo compounds and N-aryl substitution products of the 2:5-aminonaphthol-7-sulfonic acid.

- 5 7. The material dyed according to claim 1.  
8. The material dyed according to claim 2.  
9. The material dyed according to claim 3.

10. The material dyed according to claim 4.  
11. The material dyed according to claim 5.  
12. The material dyed according to claim 6. 10  
In witness whereof I have hereunto signed

my name this 12th day of May 1927.

FRITZ STRAUB: